

## UNITED STATES PATENT OFFICE

2,413,024

## PROCESS FOR FINISHING TEXTILE MATERIALS, PARTICULARLY TO RENDER THE SAME WATER REPELLENT

Ernst Zerner, Gertrude D. M. Davies, and Peter I. Pollak, New York, N. Y., assignors, by mesne assignments, to Sun Chemical Corporation, New York, N. Y., a corporation of Delaware

No Drawing. Application May 4, 1943,  
Serial No. 485,624

3 Claims. (Cl. 8—116.2)

1

The present invention relates to improvements in the treatment of textiles, in order to render such textiles repellent to water.

Different processes have been proposed for rendering textiles repellent to water in such a way that the water repellency will persist, even though the textiles be subjected to the usual cleansing methods, i. e., dry cleaning and laundering. Generally the manufacturing of products suitable for this purpose is relatively complicated and costly.

We have found that products very suitable for rendering textiles water repellent are so-called "Schiff's bases." We understand that under that term are included anilines which are condensation products of primary amines with either an aldehyde or ketone. In our process we include only those products which are made of a ketone containing an aliphatic chain of at least 8 and preferably 8 to 20 carbon atoms, and a primary amine containing either an alkyl radical having at least 8 carbon atoms or an aryl radical.

We have prepared such Schiff's bases, for instance, from di-heptadecyl ketone and aniline or alpha- or beta-naphthylamine, and also from di-heptadecyl ketone and dodecylamine.

By the term "textiles" are included cotton and jute, linen, hemp, wool, and various artificial fibers of organic material.

The textiles to be made water repellent are treated in a solution of one of these Schiff's bases in an organic solvent. After drying in the open air, or at a slightly elevated temperature, a very low or no water repellency is obtained. After baking the material at an elevated temperature of about 100–160° C. for a certain time, preferably at 150° C. for five minutes, a high water repellent effect is obtained, and textiles so treated do not lose the water repellency, at least not in a considerable percentage, by dry cleaning or laundering several times. This, in our opinion, proves that the Schiff's bases and the textiles enter some chemical reaction by which at least the superficial layers of the textiles are altered in such a way that they become repellent to water.

The following examples will illustrate the process of the present invention, although the invention is not restricted to these.

*Example 1.*—Plain weave grey cotton cloth was dipped into a 1% solution of di-heptadecyl-beta-naphthylamine anile in Stoddard solvent (white spirit), the excess of the solution was squeezed out, and the dipping and squeezing repeated. The cloth was then dried in the open air and baked for five minutes at 150° C. After simple drying without baking no water repellency was observa-

ble. After baking the cloth showed a spray rating of nearly 100, which is reduced by dry cleaning or laundering to only about 80.

The di-heptadecyl-beta-naphthylamine anile was prepared in the following way: 100 parts (by weight) of di-heptadecyl ketone and 27.8 parts of beta-naphthylamine were heated in a closed vessel for 2½ hours to 140–170° C. The compound was recrystallized once from alcohol, and had a melting point of 176–180° C., and corresponded probably to the formula:



*Example 2.*—51 parts of di-heptadecyl ketone and 19 parts of dodecyl amine, and 1 part of zinc chloride were heated in a closed vessel to 150–170° C. for 5 hours. The final product, after being recrystallized once from benzene, melted at 81–82° C., and corresponded probably to the formula:



A piece of gabardine was dipped twice into a 2% warm alcoholic solution and then squeezed, dried in the open air, and baked at 130° C. for 15 minutes. The spray rating was 100.

*Example 3.*—Instead of dissolving the compound mentioned in Example 2 in alcohol, an emulsion was made of the following composition: 1.5 parts of an emulsifier like Duponol ME and 10 parts of an aluminium acetate solution of 20% were warmed up to 80° C., and 20 parts of the compound above mentioned, and in molten condition, was poured into the mixture under vigorous agitation, and 70 parts of hot water was added. The emulsion so obtained was passed through a colloid mill.

For impregnating purposes this emulsion was diluted in a ratio of 1:20 with warm water, and the cloth to be rendered water repellent was dipped in twice, squeezed out, dried by means of a fan at 50–60° C. for five minutes, and then baked at 150° C. for another five minutes. The so-treated cotton cloth showed a spray rating of 90, and the water repellency was pretty resistant to dry cleaning and laundering.

Having thus described our invention, what we claim as new and desire to secure by Letters Patent is:

1. The process for rendering cellulosic textiles

## 3

water repellent, which includes incorporating therein a monomeric compound of the formula



in which  $R_1$  and  $R_2$  represent alkyl radicals with at least 8 carbon atoms, and  $R_3$  represents a radical selected from the group consisting of alkyl radicals having at least 8 carbon atoms and aryl radicals, drying, and baking at 130° C. to 150° C.

2. A process of rendering cellulosic textiles and

## 4

the like water repellent, which includes incorporating therein di-heptadecyl-beta-naphthylamine anile, drying, and baking at 130° C. to 150° C.

5. 3. A process of rendering cellulosic textiles and the like water repellent, which includes incorporating therein the reaction product of di-heptadecyl ketone and dodecyl amine, drying and baking at 130° C. to 150° C.

ERNST ZERNER.  
GERTRUDE D. M. DAVIES.  
PETER I. POLLAK.